# EUROPEAN PATENT SPECIFICATION

(11) **EP 2 036 634 B1**
(45) Date of publication and mention of the grant of the patent: **11.08.2010**
(21) Application number: 08252676.5
(22) Date of filing: 12.08.2008
(51) Int. Cl.: B22D 13/10

(54) **Centrifugal casting method and apparatus**
Schleudergiessverfahren und Vorrichtung
Procédé et appareil de coulage centrifuge

(30) Priority: 14.09.2007 GB 0717925
(43) Date of publication of application: 18.03.2009
(73) Proprietor: Rolls-Royce plc, 65 Buckingham Gate London SW1E 6AT (GB)
(72) Inventor: Voice, Wayne Eric, West Bridgford Notthingham, NG2 5JB (GB)
(74) Representative: Barcock, Ruth Anita

(56) References cited:
- JP-A- 8 262 008
- JP-A- 2000 024 008
- US-A- 3 364 978
- US-A- 4 162 039

## Description

This invention relates to methods and apparatus for centrifugal casting of components.

According to a first aspect of the invention there is provided a method of forming a cast component comprising the steps of: providing a chamber containing a molten alloy and an impurity and a conduit having a supply valve connecting the chamber with a mould; rotating the chamber about an axis to separate the alloy and the impurity by centrifuging; and opening the valve to supply the alloy from the chamber to the mould rotating about the axis to centrifugally cast the alloy in the mould.

Preferably the molten alloy comprises titanium, vanadium, chromium and aluminium. The molten alloy may be formed from the oxides of at least some of its constituent elements which react exothermically in the chamber. The impurity may be aluminium oxide.

The valve may be opened when a mass blocking the a conduit between the chamber and the mould melts after a predetermined period to allow the molten alloy to be supplied to the mould

According to a second aspect of the invention there is provided apparatus for forming a cast component, the apparatus comprising a chamber for holding an alloy and being rotatable about an axis, a rotatable mould rotatable about the axis, a conduit having a supply valve connecting the chamber with the mould, rotating means for rotating the chamber with a velocity sufficient to separate molten alloy from an impurity by centrifuging and for rotating the mould with sufficient velocity to centrifugally cast a component.

The conduit may have a supply valve for allowing the supply of alloy from the chamber to the mould.

Preferably the mould is annular.

Embodiments of the invention will now be described by way of example only, with reference to the accompanying drawings, in which:
Fig. 1 depicts a schematic diagram of a casting apparatus according to a first embodiment of the invention.

Figure 1 depicts a centrifugal casting apparatus in accordance with a first embodiment of the invention.

The apparatus comprises a chamber 2 and a mould 4 connected by a conduit 6. The chamber and mould are mounted together on a frame (not shown) which enables the two components to rotate about an axis 8.

An alloy is added to the chamber which must be capable of withstanding the melting point of the alloy.

The alloy may be provided as an ingot having the desired composition which is melted within the chamber. Alternatively the ingot is melted away from the chamber in a crucible or such like and added to the chamber 2 in its molten form. Additional heating elements (not shown) may be provide in or around the chamber 2 to maintain the alloy in its molten state. In the preferred embodiment, described in greater detail below, the alloy is formed during an exothermic reaction within the chamber between molten aluminium and oxides selected from titanium, vanadium and / chromium.

The alloy may contain impurities which will affect the final characteristics of the cast component. To remove these impurities the chamber 2 is rotated about the axis 8 to separate the alloy 10 from the impurity 12 centrifugally.

Once the alloy is sufficiently separated from the impurity, preferably determined empirically through trial and error, a supply valve in the conduit is opened to supply the alloy to the mould 4 for the centrifugal casting process.

In the preferred embodiment the mould 4 lies further away from the axis than the chamber 2 which allows the alloy to be supplied using the generated centrifugal force. In alternative arrangements the alloy may be pumped from the chamber to the mould.

The mould 4, like the chamber 2, rotates about the axis 8 and produces a sound, porous free casting with a fine grain size due to the relatively rapid solidification of the alloy and the centrifugal force exerted which breaks up dendrite formation whilst forming an accurate cast shape.

The mould is preferably ceramic formed using a lost wax process. In the preferred use, where the cast component is an engine casing, the mould is annular. For other, more complex shapes it will be appreciated that an appropriate mould shape is required. It may be necessary to provide a counter-balance to ensure smooth rotation of the mould about the axis.

In the preferred method the alloy comprises titanium, vanadium, chromium and aluminium. The preferred alloy has 25wt%V, 15%Cr, 2%Al with the balance being Ti plus any impurities. The preferred method of forming the alloy is to load the chamber 2 with titanium, vanadium and chromium oxides in powder, flake or particle form. Aluminium is added to the chamber in flake form and mixed with the other elements.

When the oxides of the elements combine with molten aluminium they react exothermically to give aluminium oxide Al₂O₃ and liquid alloy. The aluminium oxide is an impurity and must be removed else the final characteristic of the alloy will be affected.

The constituent oxides and aluminium flakes are placed in the chamber 2 as a charge. A mass, preferably disk shaped, and formed of the desired alloy is placed at the base of the chamber 2 to prevent the charge from entering the cast. Once the chamber is loaded with the charge rotation of the chamber and the cast about the axis 8 is started.

When the preferred rotation speed of the order 200rpm is achieved the aluminium in the chamber is heated till it is melted. This begins a self-sustaining exothermal reaction within the charge reducing the oxides to their base metals and melting further aluminium in the chamber. In an alternative technique the exothermic reaction can be started by means of an electrical resistance heating wire at the point furthest from the disk. Beneficially this technique means that the charge need not be heated en masse. The reaction propagates through the charge till all the powder or flakes have been converted to their base metals and alloyed. Sufficient aluminium flakes are provided so that once all the oxides have been reduced to their base metals a small proportion of the aluminium remains to be alloyed with the other components.

Al₂O₃ is less dense than the alloy and is squeezed to the inside of the chamber by the alloy moving outwards under the influence of the centrifugal force. The alloy may then be supplied to the mould. It typically takes less than 5 minutes for the reaction to propagate through the charge depending on the charge constituents, size of the charge and rotational speed.

When the melted alloy reaches the disk blocking the conduit 6 the heat of the alloy causes the disk to melt which allows the flow of molten alloy into the rotating cast component. The alloy continues to flow till the cast is full and it is therefore important that the volume of the cast is equal to or less than the volume of alloy formed in the chamber to stop impurities from entering the cast.

The rotational speed and density difference between the alloy and the aluminium oxide should be sufficient to allow adequate separation before the disk melts. Routine trial and error experiments may be used to determine an acceptable rotational velocity for any given alloy and charge size to ensure adequate separation of the alloy from the impurity. By changing the properties of the disk, either physically or compositionally it is possible to change the time taken for it to melt and thereby control the supply of alloy to the cast in that way.

For the alloy described above the density difference between the aluminium oxide impurity at 2.5 g/cm^3 and the alloy at around 5g/cm^3 a revolution velocity of 200 rpm is sufficient to separate the alloy and impurity.

It will be appreciated that the present invention offers significant advantages. Offering the ability to separate impurities from the alloy during the casting process enables high quality control and the use of alloy stock having higher levels of impurity. The technique enables the desired quantity of alloy to be manufactured at its point of use which overcomes the need to melt the alloy first during manufacture and again as it is used in the casting process with significant energy savings. As a further advantage the reliance on the alloy supply chain is reduced as the alloy can be made at its point of use using its constituent elements.

## Claims

1. A method of forming a cast component comprising the steps of:
providing a chamber (2) containing a molten alloy and an impurity and a conduit having a supply valve connecting the chamber with a mould;
rotating the chamber about an axis (8) to separate the alloy (10) and the impurity (12) by centrifuging; and
opening the valve to supply the alloy (10) from the chamber to the mould (4) rotating about the axis to centrifugally cast the alloy in the mould.

2. A method according to claim 1, wherein the molten alloy comprises titanium.

3. A method according to claim 2, wherein the molten alloy comprises aluminium.

4. A method according to claim 2 or claim 3, wherein the molten alloy comprises titanium, aluminium, vanadium and chromium.

5. A method according to claim 4, wherein the alloy is formed from constituent elements of titanium oxide, vanadium oxide and chromium oxide which react exothermically with the aluminium in the chamber.

6. A method according to claim 4, wherein the impurity is aluminium oxide.

7. A method according to any preceding claim, wherein the valve is opened when a mass blocking a conduit between the chamber and the mould melts after a predetermined period to allow molten alloy to be supplied to the mould.

8. Apparatus for forming a cast component, the apparatus comprising a chamber for holding an alloy and being rotatable about an axis, a mould rotatable about the axis, a conduit having a supply valve connecting the chamber with the mould, and rotating means for rotating the chamber with a velocity sufficient to separate molten alloy from an impurity by centrifuging and for rotating the mould with sufficient velocity to centrifugally cast a component.

9. Apparatus according to claim 8, wherein the supply valve comprises a mass of material blocking the conduit.

10. Apparatus according to any one of claims 8 and 9, wherein the mould is annular.

11. Apparatus according to any one of claims 8 to 10, wherein the chamber contains constituent elements of titanium oxide, vanadium oxide and chromium oxide and molten aluminium.

## Patentansprüche

1. Verfahren zur Herstellung eines Gussteiles im Schleudergießverfahren mit den folgenden Schritten:
es wird eine Kammer (2) bereitgestellt, die eine geschmolzene Legierung und eine Verunreinigung enthält, wobei eine mit einem Absperrventil ausgerüstete Leitung die Kammer mit einer Gießform verbindet;
es wird die Kammer um eine Achse (8) gedreht, um die Legierung (10) von der Verunreinigung (12) durch Zentrifugierung zu trennen; und
es wird das Ventil geöffnet, um die Legierung (10) in die um die Achse rotierende Gießform (4) im Schleuderguss einzuleiten.

2. Verfahren nach Anspruch 1, bei welchem die geschmolzene Legierung Titan enthält..

3. Verfahren nach Anspruch 2, bei welchem die geschmolzene Legierung Aluminium enthält.

4. Verfahren nach Anspruch 2 oder Anspruch 3, bei welchem die geschmolzene Legierung Titan, Aluminium, Vanadium und Chrom enthält.

5. Verfahren nach Anspruch 4, bei welchem die Legierung aus einzelnen Elementen aus Titanoxid, Vanadiumoxid und Chromoxid hergestellt wird, die exotherm mit dem Aluminium in der Kammer reagieren.

6. Verfahren nach Anspruch 4, bei welchem die Verunreinigung Aluminiumoxid ist.

7. Verfahren nach einem der vorherigen Ansprüche, bei welchem das Ventil **dadurch** geöffnet wird, dass eine Masse, die eine Leitung zwischen der Kammer und der Gießform blockiert, nach einer vorbestimmten Periode schmilzt, sodass die geschmolzene Legierung in die Gießform eingeleitet werden kann.

8. Vorrichtung zur Herstellung eines Gussteiles im Schleudergießverfahren, wobei die Vorrichtung folgende Teile aufweist: eine um eine Achse rotierbare Kammer zur Aufnahme einer Legierung; eine um die Achse rotierbare Gießform; eine mit einem Absperrventil ausgerüstete Leitung, die die Kammer mit der Gießform verbindet; und Rotationsmittel zur Drehung der Kammer mit einer Drehzahl, die groß genug ist, um die geschmolzene Legierung von einer Verunreinigung durch Zentrifugierung zu trennen und zur Drehung mit einer Drehzahl, die groß genug ist, um ein Gussteil durch Schleuderguss herzustellen.

9. Vorrichtung nach Anspruch 8 , bei welcher das Absperrventil eine Masse aus einem Material aufweist, das die Leitung blockiert.

10. Vorrichtung nach einem der Ansprüche 8 und 9, bei welcher die Gießform ringförmig ausgebildet ist.

11. Vorrichtung nach einem der Ansprüche 8-10, bei welcher die Kammer einzelne Elemente aus Titanoxid, Vanadiumoxid und Chromoxid sowie geschmolzenem Aluminium enthält.

## Revendications

1. Procédé pour former un composant moulé comprenant les étapes consistant à :
prévoir une chambre (2) comprenant un alliage en fusion et une impureté et un conduit ayant une soupape d'alimentation raccordant la chambre à un moule ;
faire tourner la chambre autour d'un axe (8) pour séparer l'alliage (10) et l'impureté (12) par centrifugation ; et
ouvrir la soupape pour alimenter l'alliage (10) de la chambre jusqu'au moule (4) tournant autour de l'axe pour mouler de manière centrifuge l'alliage dans le moule.

2. Procédé selon la revendication 1, dans lequel l'alliage en fusion comprend du titane.

3. Procédé selon la revendication 2, dans lequel l'alliage en fusion comprend de l'aluminium.

4. Procédé selon la revendication 2 ou la revendication 3, dans lequel l'alliage en fusion comprend du titane, de l'aluminium, du vanadium et du chrome.

5. Procédé selon la revendication 4, dans lequel l'alliage est formé à partir d'éléments constitutifs d'oxyde de titane, d'oxyde de vanadium et d'oxyde de cuivre, qui réagissent de manière exothermique avec l'aluminium dans la chambre.

6. Procédé selon la revendication 4, dans lequel l'impureté est de l'oxyde de l'aluminium.

7. Procédé selon l'une quelconque des revendications précédentes, dans lequel la soupape est ouverte lorsqu'une masse bloquant un conduit entre la chambre et le moule fond après une période prédéterminée pour permettre à l'alliage en fusion d'être alimenté au moule.

8. Appareil pour former un composant moulé, l'appareil comprenant une chambre pour contenir un alliage et pouvant tourner autour d'un axe, un moule pouvant tourner autour de l'axe, un conduit ayant une soupape d'alimentation raccordant la chambre au moule, et des moyens de rotation pour faire tourner la chambre avec une vitesse suffisante pour séparer l'alliage en fusion d'une impureté par centrifugation, et pour faire tourner le moule avec une vitesse suffisante pour mouler de manière centrifuge un composant.

9. Appareil selon la revendication 8, dans lequel la soupape d'alimentation comprend une masse de matériau bloquant le conduit.

10. Appareil selon l'une quelconque des revendications 8 et 9, dans lequel le moule est annulaire.

11. Appareil selon l'une quelconque des revendications 8 à 10, dans lequel la chambre contient des éléments constitutifs d'oxyde de titane, d'oxyde de vanadium et d'oxyde de chrome et de l'aluminium en fusion.
